

## UNITED STATES PATENT OFFICE

2,673,161

## CORROSION INHIBITING COMPOSITION

Edgar A. Dieman, Crown Point, Ind., assignor to  
Standard Oil Company, Chicago, Ill., a corpora-  
tion of Indiana

No Drawing. Application November 27, 1951,  
Serial No. 258,501

11 Claims. (Cl. 106—14)

1

This invention relates to improvements in corrosion inhibiting compositions otherwise known as slushing compounds, and more particularly is directed to corrosion inhibiting compositions for protecting metal surfaces, particularly those of ferrous and related metal or alloy products from rusting and from the corrosive action of air or oxygen in the presence of moisture or other aqueous liquids.

Metal surfaces whenever possible are protected from corrosion and/or rusting by a coating of some kind. In general, two types of protective coatings have been employed, namely permanent and temporary coatings. In the first class are included oxide coatings, phosphate coatings, paints, varnishes and other non-metallic materials which form dry, hard films. In the second class of protective coatings which are of the type which must at some time be readily removed from the surfaces they are protecting are those products prepared from oleaginous materials, such as petroleum oils, petrolatums, waxes, greases, asphalts, etc. While such products give satisfactory protection under certain conditions, under many conditions they do not provide the protection desired, and require the addition thereto of rust and/or corrosion inhibitors. Anti-rust or slushing compositions are used for the protection of metals either in the form of stock or fabricated articles against corrosion and/or rusting. Materials prior to storage should be coated with an anti-rust material to prevent corrosion and/or rusting while in storage; and finished or semi-finished metal stocks destined for shipment by rail or by water must be protected against attack by moisture by coating such materials with suitable anti-rust or slushing compounds. Materials for shipment overseas must be protected against attack by salt spray.

It is an object of the present invention to provide anti-rust compositions which will effectively prevent and/or inhibit corrosion of metal surfaces. Another object of the present invention is to provide improved slushing and/or anti-rust compositions.

In accordance with the present invention, the foregoing objects can be attained by employing as the slushing composition an oleaginous material containing in combination from about 0.5% to about 10% of an alkali metal soap of a preferentially oil-soluble sulfonic acid, and from about 0.5% to about 25% of the polymeric residue that is produced in hydrocarbon synthesis from hydrogen and carbon monoxide in the presence of an iron catalyst, or the alkali metal and/or alka-

2

line earth metal soaps thereof, such as the sodium, lithium, calcium, barium, strontium soaps or mixtures thereof.

The hydrocarbon synthesis, from which the polymeric residue of the present invention are obtained, is usually performed at temperatures from about 390° F. to about 660° F., and under superatmospheric pressures from slightly in excess of atmospheric to as high as 600 pounds per square inch gauge. An increased yield of the polymeric residue is produced when the aforementioned iron catalyst contains an alkali metal oxide or carbonate promoter.

The aforesaid polymeric residue is produced as a primary condensate from the condensable gases that are manufactured in the described hydrocarbon synthesis process or it can be a residue from a fractional distillation of liquid product therefrom or it can constitute a mixture of the two. These polymeric residues have a pour point of substantially room temperature and comprise a mixture of about 85-90% by weight of heavy hydrocarbons and oxygenated compounds, a high proportion of which is unsaturated. Of the hydrocarbons some 20 to 30 percent are paraffinic, and the remaining 70 to 80 percent are olefinic. A very considerable portion of the olefins are mono-olefins. The polymeric residue is soluble in 50-50 benzol-acetone, and ranges in carbon number from about C<sub>11</sub> to C<sub>35</sub>, and perhaps, to a minor extent, somewhat higher. The product contains about 10 to 15 per cent oxygenated compounds, including alcohols, aldehydes, acids, esters and ketones. Normally, about 5 percent and a maximum of 10 percent of the hydrocarbons are normal paraffins, the branching of the chains being largely methyl groups and increasing in number of branched chains per molecule with increase in molecular weight. At least about 25%, by weight, of the polymeric residue consists of said oxygenated compounds and hydrocarbons that melt between about 120° F.-212° F.

Illustrative of a method of obtaining the polymeric residue used in the present invention, carbon monoxide and hydrogen is reacted in the presence of an alkylated iron catalyst at a temperature of 600° F. to 650° F., under a pressure of 250 pounds per square inch, and at 2:1 recycle ratio. The fluidized catalyst used consists of an equilibrium mixture of metallic iron and iron oxide upon which was deposited 0.47%, by weight, of K<sub>2</sub>O. A primary condensate referred to as gas oil, constituting about 3.9% of the total weight balance in synthesis was recovered from the product gases. A portion of the product was

recovered by initial condensation at high temperature and the remainder obtained as a residue from the distillation of the liquid hydrocarbons. By mixing the products so obtained in the proportions of their initial formation, a polymeric residue product having a melting point slightly above room temperature, is obtained.

A typical polymeric residue had the following distillation characteristics and neutralization values:

| Percent Collected                   | ° F.     | Neutralization No.<br>(MgKOH/gram) |
|-------------------------------------|----------|------------------------------------|
| 10%                                 | 400-450  | 20.1                               |
| 20%                                 | 450-480  | 12.8                               |
| 30%                                 | 480-500  | 10.4                               |
| 40%                                 | 500-530  | 13.2                               |
| 50%                                 | 530-570  | 14.6                               |
| 60%                                 | 570-585  | 18.7                               |
| 67.5%                               | 585-590  | 28.3                               |
| Residue                             | Over 590 | 4.4                                |
| Neutralization No. of Total Product |          | 10.8                               |

The polymeric residue can be used as such in combination with the alkali metal soaps of the preferentially oil-soluble petroleum sulfonic acids; however, I prefer to use the alkali metal and/or alkaline earth metal soaps of such polymeric residues. These soaps can be readily prepared by reacting the polymeric residue with a sufficient amount of an alkali metal hydroxide or an alkaline earth hydroxide to neutralize the acidity of the polymeric residue at a temperature of from about 200° F. to about 325° F., and the soaps recovered by extraction with a suitable solvent such as a low boiling hydrocarbon, for example, hexane, naphtha, etc.

The preparation of the calcium soap of the polymeric residue is illustrated by the following example:

To 200 grams of polymeric residue, was added about 100 grams of 75% ethyl alcohol-water solution to act as solvent during the process of neutralization. 40 1.65 grams (which is about 10% in excess of the calculated amount necessary) of calcium hydroxide was made into a slurry with water and slowly added to the polymeric residue-alcohol and water solution while it was stirred with a mechanical mixer at 150° F. After all the  $\text{Ca}(\text{OH})_2$  slurry had been added, mixing and heating was continued at temperatures sufficient to boil off the alcohol and finally the water. The temperature of the mix was raised to 230° F. at which point the last of the water was evaporated and the product made substantially dry. The product was then cooled to room temperature and dissolved in about 2 volumes of hexane. The insoluble portion and unreacted calcium hydroxide was separated by centrifuging from which 6.5% was recovered as insoluble material. The hexane soluble material was decanted off and the hexane evaporated. This portion amounted to 89.5% of the sample making a total recovery of 93% oil-soluble sulfonic acids.

The alkali metal soaps of the preferentially oil-soluble sulfonic acids used in the present invention include such soaps of alkyl sulfonic acids, petroleum sulfonic acids, alkaryl sulfonic acids and aralkyl sulfonic acids, although I prefer to use the alkali metal soaps of the so-called mahogany acids obtained in the treatment of hydrocarbon oils with strong sulfuric acid of at least about 95% strength, usually fuming sulfuric acid. These mahogany acids have molecular weights of from about 410 to about 500. The method of obtaining alkali metal soaps of the so-called

mahogany acids, well known to those acquainted with the petroleum refining art, is illustrated by the following example, which describes the preparation of the sodium soap.

5 A petroleum oil distillate having a Saybolt Universal viscosity at 100° F. of from about 200 seconds to about 850 seconds is treated with from about 7 to about 8 pounds of fuming sulfuric acid per gallon of oil in one-half pound increments or "dumps." After the acid sludge from each one-half pound acid "dump" is settled and withdrawn, the next one-half pound of fuming sulfuric acid is added to the oil. The temperature of the oil before the fuming sulfuric acid is added thereto is maintained below about 60° F., but due to the heat of the reaction upon the addition of the sulfuric acid, the temperature of the oil may rise to from about 90° F. to about 100° F. After the required total amount of fuming sulfuric acid has been added to the oil and the oil freed of acid sludge, the acid-treated oil containing oil-soluble sulfonic acids dissolved therein, is neutralized with a solution of sodium hydroxide. The aqueous alkali solution is then separated from the oil solution containing dissolved therein sodium soap of sulfonic acids and the latter is then separated from the oil by extraction with alcohol of about 60% strength. The alcohol layer containing dissolved sodium sulfonates is then separated from the oil and subsequently distilled to recover the alcohol and remove water. The crude sulfonic soap obtained in this manner contains from about 30% to about 60% sodium sulfonate, from about 30% to about 60% oil, from about 1% to about 10% water, and up to 10% inorganic salts which may be removed by the procedure hereinafter described.

The above procedure may be modified in that after the acid sludge is removed from the acid-treated oil, the oil containing dissolved sulfonic acids is extracted with about 60% alcohol to remove the sulfonic acids which may then be neutralized with sodium hydroxide and subsequently freed of the alcohol by distillation.

The crude soaps of these preferentially oil-soluble sulfonic acids obtained by the procedure described above may be freed of inorganic salts by purification. This purification is preferably accomplished by dilution of the crude soap with from about 1/2 to about 10 parts, preferably 1 to 2 parts of 50%, or higher strength alcohol, preferably alcohol of 60 to 70% strength, and allowing the salts to settle while maintaining the mixture within the temperature range of 130° F. to 175° F., preferably 155° F. to 165° F. When the salts have settled the supernatant alcohol-soap layer is separated and the alcohol is recovered by conventional distillation procedure. By this method of purification, the salt content of the crude sulfonic soap can be readily reduced to 5%, or less, e. g., to about 3.5%. To facilitate handling, the sulfonates are preferably dissolved in a petroleum oil to give a blend containing about 35-50% sulfonate.

Although in the above example, an oil of 200 seconds to 850 seconds Saybolt Universal viscosity at 100° F. has been used, it is to be understood that the petroleum sulfonic acids can be obtained by the treatment of petroleum distillates having Saybolt Universal viscosities at 100° F., ranging from about 50 seconds to about 1000 seconds, or higher. Furthermore, the sulfuric acid employed can range from about 3 to about 9 pounds per gallon of oil.

The vehicle for the herein-described inhibitors

can be any of the materials usually used as the base for such compositions. These are usually natural or synthetic hydrocarbon oils covering wide range of viscosities, such as petroleum distillates of relatively low viscosity to distillates or residuums of high viscosities. Solid and semi-solid petroleum products such as waxes and petrolatums can also be employed. Also waxes and oils of animal, vegetable or marine origin, or mixtures of these with hydrocarbon oils and waxes can be used as the base material. To facilitate application, the composition may be thinned with a volatile solvent, such as a low boiling hydrocarbon naphtha, etc.

The effectiveness of the herein described composition in inhibiting corrosion is demonstrated by the data in the following table. These data were obtained by subjecting steel test panels coated with the various compositions to the humidity cabinet test and the time before rusting occurs noted in each instance.

In the humidity test the steel panels are suspended in a special cabinet described in the National Military Establishment specification designated JAN-H-792(6-21-49), and the time of initial corrosion of the panels noted. The humidity cabinet is provided with heating units and thermal regulators for automatic temperature control. A water level is maintained in the bottom of the cabinet to give approximately 100% humidity at all times. The steel panels are coated by dipping into the rust preventive material and are suspended in the cabinet by stainless steel or Monel hooks. The JAN-H-792 specification is modified to the extent that a temperature of 100° F. ( $\pm 2$ ° F.) instead of 120° F. ( $\pm 2$ ° F.) is maintained in the cabinet, and from 1 to 1.5 complete changes of saturated air per hour are provided in the cabinet, instead of 8 ( $\pm 1$ ) linear feet per hour.

| Run No. | Blend                                                                                                                             | Hours in Humidity Cabinet Before Rusting Occurred |
|---------|-----------------------------------------------------------------------------------------------------------------------------------|---------------------------------------------------|
| I       | 98% Paraffinic Oil*<br>2% Sodium Mahogany Soap                                                                                    | 72.                                               |
| II      | 94% Paraffinic Oil<br>6% Sodium Mahogany Soap                                                                                     | 72.                                               |
| III     | 94% Paraffinic Oil<br>6% Calcium Soap of Polymeric Residue                                                                        | 8.                                                |
| IV      | 92% Paraffinic Oil<br>6% Calcium Soap of Polymeric Residue<br>2% Sodium Mahogany Soap                                             | 350.                                              |
| V       | 92% Paraffinic Oil<br>6% Polymeric Residue (Unneutralized)<br>2% Sodium Mahogany Soap<br>* Control                                | 96.<br>Less than 8.<br>Do.                        |
| VI      | 25% Paraffinic Oil<br>75% SAE 50 Oil                                                                                              | 132.                                              |
| VII     | 98% No. VI<br>2% Sodium Mahogany Soap                                                                                             | Less than 8.                                      |
| VIII    | 94% No. VI<br>6% Calcium Soap of Polymeric Residue                                                                                | 240.                                              |
| IX      | 92% No. VI<br>2% Sodium Mahogany Soap<br>6% Calcium Soap of Polymeric Residue                                                     | Less than 8.                                      |
| X       | 94% No. VI<br>6% Barium Soap of Polymeric Residue<br>92% No. VI<br>2% Sodium Mahogany Soap<br>6% Barium Soap of Polymeric Residue | 156.                                              |
| XI      |                                                                                                                                   |                                                   |

The synergistic effect of the combination of the sodium mahogany soap and the alkaline earth soaps of the polymeric residue is demonstrated by comparison of runs I and III with runs IV and VI, VII, VIII and X, with runs IX and XI. Run V illustrates the effectiveness of the combina-

tion of mahogany soap and the unneutralized polymeric residue.

Similar results are obtainable with other alkaline earth and alkali metal soap of the polymeric residue and other alkali metal sulfonates. In general, however, the alkali metal soaps of the polymeric residue are somewhat less effective than the alkaline earth soaps of such residues.

Polymeric residue from the same source of the polymeric residue used in the above experiments was distilled to obtain a 60% overhead fraction and a 40% bottoms. A portion of the latter was neutralized to obtain the calcium soap thereof, and the following blends tested for their rust inhibiting properties.

| Run No. | Blend                                                              | Hours in Humidity Cabinet Before Rusting |
|---------|--------------------------------------------------------------------|------------------------------------------|
| XII     | Paraffin Oil                                                       | Less than 8.                             |
| XIII    | 94% No. XII<br>6% Calcium Soap of 40% Bottoms of Polymeric Residue | 8.                                       |
| 25      | 94% No. XII<br>4% Calcium Soap of 40% Bottoms of Polymeric Residue | 375.                                     |
| XIV     | 2% Sodium Mahogany Soap                                            | 160.                                     |
| XV      | 94% No. XII<br>6% Unneutralized 40% Bottoms of Polymeric Residue   | 8.                                       |
| XVI     | 94% No. XII<br>4% Unneutralized 40% Bottoms of Polymeric Residue   | 160.                                     |
| XVII    | 2% Sodium Mahogany Soap                                            | 72.                                      |

The mahogany soaps used in the above tables were blends of 50% soap and 50% petroleum oil.

While the herein-described invention finds its primary use in the protection of metal surfaces of metal articles in storage, stand-by equipment, etc. is also applicable to the protection of metal surfaces of equipment while in service, such as engines, machinery, etc. For such services it may be desired to incorporate in such compositions other additives, such as for example, polymeric thickeners, V. I. improvers, oiliness agents, pourpoint depressors, antioxidants, etc.

Percentages given herein and in the appended claims are weight percentages unless otherwise stated.

Although the present invention has been described by reference to specific embodiments thereof, these are given by way of illustration only and the invention is not to be limited thereto, but includes within its scope such modifications and variations as come within the spirit of the appended claims.

I claim:

1. A composition comprising a major proportion of an oleaginous material, from about 0.5% to about 10% of an alkali metal soap of a preferentially oil-soluble sulfonic acid and from about 0.5% to about 25% of a soap selected from the group consisting of an alkali metal soap, an alkaline earth metal soap and mixtures thereof, of the acidic constituents of a polymeric residue directly obtained as a product of the synthesis of liquid hydrocarbons from carbon monoxide and hydrogen at a temperature between about 390° F. and 660° F. at superatmospheric pressure in the presence of an alkalinized iron catalyst, said polymeric residue consisting predominantly of saturated and olefinic hydrocarbons, and oxygenated organic compounds having between about 11 to about 35 carbon atoms per molecule, and contains at least 25%, by weight, of a mix-

7  
ture of hydrocarbons and oxygenated organic compounds melting between about 50° C. and 100° C.

2. A composition as described in claim 1 in which the preferentially oil-soluble sulfonic acid is a preferentially oil-soluble petroleum sulfonic acid obtained from the treatment of a hydrocarbon oil with strong sulfuric acid.

3. A composition as described in claim 1 in which the alkali metal soap of a preferentially oil-soluble sulfonic acid is the sodium soap.

4. A composition as described in claim 1, in which the alkali metal soap of a preferentially oil-soluble sulfonic acid is the lithium soap.

5. A composition as described in claim 1 in which the alkali metal soap of the polymeric residue is the sodium soap.

6. A composition as described in claim 1 in which the alkaline earth metal soap of the polymeric residue is the calcium soap.

7. A composition as described in claim 1 in which the alkaline earth metal soap of the polymeric residue is the barium soap.

8. A composition as described in claim 1 in which the oleaginous material is a normally liquid hydrocarbon.

9. A composition as described in claim 1 in which the oleaginous material is a petroleum oil.

10. A slushing composition comprising a major proportion of a normally liquid hydrocarbon, from about 0.5% to about 10% of an alkali metal soap of a preferentially oil-soluble petroleum sulfonic acid and from about 0.5% to about 25% of an alkaline earth metal soap of the acidic constituents of a polymeric residue comprising a mixture of about 85% to 90%, by weight, of hy-

drocarbons, said hydrocarbons being about 70% to 80%, by weight, olefinic, and from about 10% to about 15%, by weight, oxygenated organic compounds having between about 11 to 35 carbon atoms per molecule, at least 25% by weight of the mixture of hydrocarbons and oxygenated organic compounds melting between about 120° F. to about 212° F., said polymeric residue being directly obtained as a product of the synthesis of liquid hydrocarbons of carbon monoxide and hydrogen in the presence of an alkalinized iron catalyst at a temperature between about 390° F. and 660° F., and at superatmospheric pressure.

11. A slushing composition comprising a major proportion of a hydrocarbon oil, from about 0.5% to about 10% of an alkali metal soap of a preferentially oil-soluble petroleum sulfonic acid and from about 0.5% to about 25% of an alkaline earth metal soap of the acidic constituents of a polymeric residue that consists predominantly of saturated and olefinic hydrocarbons and oxygenated organic compounds having between about 11 to about 35 carbon atoms per molecule, at least 25% by weight, of the mixture of hydrocarbons and oxygenated organic compounds having a melting point between about 120° F. and 212° F., said polymeric residue being obtained directly as a product of the synthesis of liquid hydrocarbons from carbon monoxide and hydrogen at a temperature between about 390° F. and 660° F., at superatmospheric pressure in the presence of an alkalinized iron catalyst.

EDGAR A. DIEMAN

No references cited.